

# UNITED STATES PATENT OFFICE.

ALBERT L. MARSH, OF DETROIT, MICHIGAN, ASSIGNOR TO HOSKINS MANUFACTURING COMPANY, OF DETROIT, MICHIGAN, A CORPORATION OF MICHIGAN.

## ELECTRICAL RESISTANCE ELEMENT.

1,057,755.

Specification of Letters Patent.

Patented Apr. 1, 1913.

No Drawing.

Application filed September 30, 1912. Serial No. 723,195.

*To all whom it may concern:*

Be it known that I, ALBERT L. MARSH, a citizen of the United States, residing at Detroit, in the county of Wayne and State 5 of Michigan, have invented a new and useful Improvement in Electrical Resistance Elements, of which the following is a specification.

My invention relates to an electrical resistance element adapted for general use, but more especially for use in heating appliances. For this use, the first requirement is durability, and it is with the greatest difficulty that durability can be predetermined, 15 although it can readily be discovered by actual test.

I have discovered by test that in general metals of the eighth group, fourth series, of the elements as classified by Mendeléeff in 20 the periodic system of elements, (that is, iron, cobalt and nickel) when alloyed with silicon, give rise to materials having the property of great durability under the conditions of use.

25 In practice, I prefer to use the metal nickel, alloyed with silicon in the proportion of about 5 per cent. of silicon. I have succeeded in rolling alloys running as high as 7 per cent. silicon with nickel, although the 30 alloy is so hard as to interfere somewhat with the facility of the operation. The art of rolling and drawing metals is advancing rapidly, however, and it is probable that higher percentages can be rolled in the future as the art develops.

Cobalt is generally interchangeable with nickel for the purpose intended, as I have determined by long experience and testing resistance elements of various compositions.

40 The principal difference between the two consists in the fact that cobalt alloys work easier hot and nickel alloys work easier cold. Iron, when alloyed alone with silicon, in the proportions mentioned, or in fact in any

45 proportions where the silicon shows its effects in increasing durability, is so brittle that I have not succeeded in rolling it but mixtures of iron with cobalt or nickel, or

both can be worked readily when alloyed with silicon in the proportions named. In 50 fact, the difference between the three metals—iron, cobalt and nickel—when alloyed with silicon for the purpose intended, lies principally in the ease with which a resistance element can be manufactured from 55 them, and not those properties inherent in the alloy which become important in the use of the element.

My preferred element, formed as above mentioned, has a resistivity of approximately 37 microhms per centimeter cube, which is quite high enough for convenient manufacture of translators, although not as high as some elements available on the market and, although I have not tested the resistivity of all the mixtures possible of the several metals specified, it is highly probable that the mixtures of the metals iron, nickel and cobalt, or some of them, when alloyed with silicon in the percentages 65 named, will give still higher resistances. For instance, nickel alloys in which the nickel is 30 per cent. are known to give resistivities of approximately 85 microhms per centimeter cube, and while the addition of 70 the silicon will greatly augment the durability of such an alloy, as I have discovered, it doubtless will not greatly decrease the resistivity, and may somewhat increase it. It will, of course, be understood that deoxidizers, such as manganese, may be used, in addition to the metals herein specified, for 75 its ordinary purposes, and I find that when added in a slight excess, it does not injuriously affect the alloy or the element formed 80 therefrom, but on the contrary, a slight excess when added to the nickel silicon alloy makes working easier. However, with the cobalt silicon alloy I do not find it necessary 85 to use the excess manganese.

I claim as new and desire to secure by Letters Patent—

1. An electric resistance element composed of metal of the eighth group, fourth series, mendeléeff's table, and silicon.
2. An electric resistance element composed

90

95

of metal of the eighth group, fourth series, Mendeléeff's table, and silicon, the silicon in the quantity of approximately 5 per cent.

- 3. An electric resistance element formed of an alloy of nickel and silicon.
- 4. An electric resistance element formed of an alloy of nickel and silicon, the silicon

in the proportion of approximately 5 per cent.

ALBERT L. MARSH.

In presence of—  
J. G. ANDERSON,  
J. LANDESMAN.